

1

3,230,076  
METAL REFINING PROCESS

John L. Benham, Lewiston, Louis R. Matricardi, Tonawanda, and Charles H. Weaver, Niagara Falls, N.Y., assignors to Union Carbide Corporation, a corporation of New York  
No Drawing. Filed Mar. 5, 1963, Ser. No. 262,826  
2 Claims. (Cl. 75—82)

The present invention relates to the refining of alloys to recover valuable constituents thereof. More particularly, the present invention relates to the processing of nickel base and cobalt base alloys to eliminate minor alloying constituents therefrom without significant loss of nickel or cobalt.

A wide variety of so-called high-temperature resistant alloys have been developed for use in gas turbines, exhaust gas-driven turbines and compressors, and similar devices where high tensile strength and minimum creep are required at temperatures on the order of 1500 to 1800° F. These alloys are generally based on nickel or cobalt or combinations of the two metals strengthened by additions of other metals such as chromium, molybdenum, tungsten, columbium, and may contain various amounts of iron. Some of these alloys are strengthened by precipitation hardening, the precipitate being formed either from two or more of the above-named elements or from additional elements such as titanium, aluminum, boron, and the like. In addition, such alloys usually contain carbon, silicon, and manganese.

In spite of the excellent properties of these alloys, service life is limited and consequently, considerable quantities of used metal have been accumulated. Because of the high economic value of the base metals contained in these alloys, there is considerable inducement to develop means for converting the scrap to useful form.

The aforementioned type of alloys most often cannot be reused without prior refining due to the unpredictable and uncontrollable recovery of some of the constituents, and also because some of the minor alloy constituents are not desired in all the products that might be made from this source of metal.

In general, it is desired to recover the maximum possible amount of the nickel, cobalt, chromium and molybdenum and eliminate or materially reduce the content of the remaining elements. At times, however, it is desired to also eliminate chromium and molybdenum from nickel and cobalt base alloys.

One approach to the problem has been to attempt selective oxidation of the undesired elements by blowing the molten metal with oxygen. This resulted in almost complete oxidation and removal of tungsten, columbium, molybdenum, and chromium. About half of the iron was removed by this procedure which is not always desirable. This work was reported by the U.S. Bureau of Mines in R.I. 5786. An attempt to use this process to refine a nickel-cobalt-chromium-molybdenum alloy resulted in excessive loss by oxidation of chromium and molybdenum. Also, the operating costs of this technique are not always favorable.

It is therefore an object of the present invention to provide a relatively simple and economical process for recovering nickel, cobalt and other valuable constituents from nickel and cobalt base alloys.

Other objects will be apparent from the following description and claims.

It has been discovered, as a part of the present invention, that by preparing a fused mixture of the alloy to be refined with basic slag and a selected metal oxide, e.g. chromium oxide, and reacting the selected metal oxide with the alloy, that alloy constituents such as titanium,

2

aluminum, silicon, vanadium, zirconium, columbium, tantalum, boron and carbon can be eliminated from the alloy.

It has also been discovered that chromium, in addition to the aforementioned alloy constituents, can also be removed from nickel and cobalt base alloys when iron oxide is used as the selected metal oxide.

It has further been discovered that molybdenum can also be removed from nickel and cobalt base alloys, in addition to chromium and the other specified alloy constituents, by using nickel oxide as the selected metal oxide.

In the practice of the present invention, a basic slag is melted in a refractory lined arc furnace and a mixture of the alloy to be refined and the selected metal oxide is added in increments and the resultant fused mixture is heated until evidence of reaction has ceased. In the course of the reaction, the undesired alloy constituents are oxidized by reaction with the selected metal oxide and go into the slag. The slag is then decanted and the refined metal is cast into suitable molds.

In the present invention, the slag together with the selected metal oxide addition should be basic and the amount of the slag should be approximately 0.80 to 1.25 by weight of the weight of the final alloy product. Slags which are particularly suitable for the practice of the present invention are those derived as by-products of aluminum reduction operations. These slags usually contain CaO, Al<sub>2</sub>O<sub>3</sub> and MgO in about the following proportions:

|    |                                |          |
|----|--------------------------------|----------|
| 30 | CaO                            | 25 to 50 |
|    | Al <sub>2</sub> O <sub>3</sub> | 40 to 70 |
|    | MgO                            | 1 to 15  |

The amount of selected metal oxide used in the practice of the present invention should contain at least the stoichiometric amount of oxygen necessary to completely oxidize the alloy constituents which are to be removed. Preferably, an excess of selected metal oxide is used containing on the order of 1.5 to 4 times the amount of oxygen necessary to oxidize the undesired alloy constituents.

In the present invention, when refining a chromium containing nickel or cobalt base alloy, and it is desired to retain the chromium in the alloy, chromium oxide, Cr<sub>2</sub>O<sub>3</sub>, is used as the selected metal oxide. With the use of chromium oxide in the manner of the present invention, alloy constituents such as titanium, vanadium, columbium, tantalum, boron, carbon, aluminum and silicon can be removed from the alloy. Cobalt, nickel, molybdenum and tungsten are substantially unaffected and are recovered in the refined alloy product.

Chromium oxide can also be used as the selected metal oxide in treating a chromium-free alloy when a chromium content is acceptable in the refined alloy.

When it is desired to eliminate chromium from nickel or cobalt base alloys, in addition to the previously mentioned alloy constituents, viz Ti, V, Cb, Ta, B, C, Al, Si, or when a chromium content is not desired in the refined alloy, iron oxide is used as the selected metal oxide.

Nickel oxide can be used as the selected metal oxide, with or in place of iron oxide, when it is desired to provide a molybdenum depleted alloy. That is, nickel oxide can be used to remove chromium and molybdenum, in addition to the previously mentioned minor alloy constituents which are removed through the use of iron oxide.

With regard to any iron and manganese constituents in the treated alloy, it has been found that the recovery of these materials varies with the basicity of the slag used, the recoveries increasing with increasing basicity of the slag.

The following examples are provided to further illustrate the refinement of nickel and cobalt base alloys in ac-

cordance with the present invention. For purposes of the present invention, nickel base and cobalt base alloys are those in which the sum of the nickel and cobalt contents represents a predominant proportion of the alloy.

#### EXAMPLE I

Six hundred pounds of  $\text{CaO}-\text{Al}_2\text{O}_3-\text{MgO}$  slag were melted in a refractory lined arc furnace. A mixture of the metal to be refined and chromium oxide was added incrementally to the molten slag and the resultant molten mixture was heated at a temperature of about 1700–1800° C. until all evidence of reaction ceased which took about one hour. The total amount of metal added was 1000 lbs. and the total amount of chromium oxide added was 300 lbs.

After cessation of reaction in the molten mixture, the slag was decanted and the refined metal was cast into pig molds.

The slag and metal compositions are set forth below:

#### Starting slag (including $\text{Cr}_2\text{O}_3$ addition)

|                                        | Percent |
|----------------------------------------|---------|
| $\text{CaO}$                           | 34.5    |
| $\text{Al}_2\text{O}_3$                | 26.4    |
| $\text{MgO}$                           | 2.1     |
| $\text{Cr}_2\text{O}_3$ <sup>1</sup>   | 34.9    |
| $\text{SiO}_2$ , $\text{TiO}_2$ , etc. | Balance |

<sup>1</sup> Specification of chromium oxide used:

|                  | percent, min. | percent, max. |
|------------------|---------------|---------------|
| Cr               | 67            | 67            |
| S                | 0.2           | 0.2           |
| C                | 0.05          | 0.05          |
| Fe               | 0.01          | 0.01          |
| Loss on ignition | 0.5           | 0.5           |

|    | Original Alloy Composition (Weight 1,000 lbs.), Percent | Refined Alloy Composition—Weight*, Percent |
|----|---------------------------------------------------------|--------------------------------------------|
| Ni | 54.30                                                   | 53.86                                      |
| Co | 17.80                                                   | 20.74                                      |
| Cr | 14.83                                                   | 18.58                                      |
| Mo | 4.44                                                    | 4.67                                       |
| Fe | 1.17                                                    | 1.84                                       |
| Al | 4.09                                                    | 0.04                                       |
| Cu | 0.03                                                    |                                            |
| Si | 0.39                                                    | 0.03                                       |
| Ti | 1.21                                                    | 0.11                                       |
| O  | 0.16                                                    | 0.053                                      |
| P  |                                                         | 0.018                                      |
| S  |                                                         | 0.016                                      |
| O  |                                                         | 0.07                                       |
| H  |                                                         | 0.001                                      |
| N  |                                                         | 0.01                                       |

\*735 lbs. were recovered as cast pigs; the skull left in the furnace (which can be recovered) was not weighed.

#### Final slag

|                         | Percent |
|-------------------------|---------|
| $\text{CaO}$            | 31.6    |
| $\text{Al}_2\text{O}_3$ | 32.4    |
| $\text{Cr}_2\text{O}_3$ | 23.6    |
| $\text{MgO}$            | 7.3     |
| $\text{SiO}_2$          | 0.9     |
| $\text{TiO}_2$          | 2.1     |

The product obtained was eminently suited for reuse in the preparation of other alloys containing nickel, cobalt, chromium, and molybdenum.

#### EXAMPLE II

One hundred fifty pounds of Ni—Co—Cr—Mo alloy were melted in a magnesia-lined electric tilting furnace under a slag made up of mill scale, silica sand, lime, and black nickel oxide. The approximate weight of the slag was 212 lbs. per batch; the metal weight per batch was 150 lbs. The temperature of the molten material was about 1600–1700° C. While all the materials were molten, the contents of the furnace were poured into a pot and the slag and metal phases were separated after reaction had ceased, which took about 1 hour.

The composition of the starting and final materials is set forth below:

#### Starting mixture

|                                              | Pounds |
|----------------------------------------------|--------|
| 5 Ni—Co—Cr—Mo alloy                          | 150    |
| Dried mill scale ( $\text{Fe}_3\text{O}_4$ ) | 150    |
| Black nickel oxide                           | 12     |
| Lime                                         | 25     |
| Silica sand                                  | 25     |

10

#### Mill scale

|                | Percent |
|----------------|---------|
| Fe             | 73.61   |
| $\text{SiO}_2$ | 0.24    |
| $\text{MnO}$   | 0.74    |
| C              | 0.17    |

15

#### Black nickel oxide

|       | Percent |
|-------|---------|
| 20 Ni | 76.18   |
| Co    | 0.02    |
| Fe    | 0.60    |
| Si    | 0.09    |

25

| Starting Metal (150 lbs.) | Percent | Refined Metal (150 lbs.) | Percent |
|---------------------------|---------|--------------------------|---------|
| Ni                        | 47.82   | Ni                       | 46.14   |
| Co                        | 28.23   | Co                       | 25.96   |
| Cr                        | 14.85   | Cr                       | 0.38    |
| Mo                        | 3.60    | Mo                       | 1.84    |
| Cu                        | 0.20    | Cu                       |         |
| Fe                        | 1.51    | Fe                       | 25.34   |
| C                         | 0.61    | C                        | 0.01    |
| Al                        | 1.03    | Al                       | <0.02   |
| Ti                        | 1.90    | Ti                       | <0.02   |

35

#### Final slag

|       | Percent |
|-------|---------|
| Cr    | 9.52    |
| Mo    | 1.48    |
| Fe    | 29.88   |
| 40 Ni | 4.86    |

45

What is claimed is:

1. A process for refining nickel base and cobalt base alloys by removing minor alloying constituents therefrom including titanium, aluminum and silicon, said process comprising providing a fused mixture of the alloy to be treated with a basic slag and chromium oxide; and reacting said chromium oxide with the admixed alloy to cause oxidation and removal of minor alloy constituents including titanium, aluminum and silicon.

2. A process for refining nickel base and cobalt base alloys which contain minor proportions of at least one metal selected from the group consisting of titanium and silicon, said process comprising providing a fused mixture of the alloy to be treated with a basic slag and chromium oxide; and reacting said chromium oxide with the admixed alloy to cause oxidation and removal of said selected metal.

#### References Cited by the Examiner

##### UNITED STATES PATENTS

|           |        |           |       |
|-----------|--------|-----------|-------|
| 1,218,412 | 3/1917 | Kissock   | 75—84 |
| 1,552,609 | 9/1925 | Hybinette | 75—82 |
| 1,674,438 | 6/1928 | Hybinette | 75—82 |
| 2,049,721 | 8/1936 | Perrin    | 75—82 |
| 2,902,359 | 9/1959 | Schott    | 75—82 |
| 3,030,201 | 4/1962 | Queneau   | 75—82 |

##### FOREIGN PATENTS

70 117,719 11/1943 Australia.

HYLAND BIZOT, Primary Examiner.

BENJAMIN HENKIN, Examiner.